

## UNITED STATES PATENT OFFICE

1,942,150

## ALLOY FOR SURGICAL NEEDLES

Wilhelm Rohn, Hanau-on-the-Main, Germany

No Drawing. Application July 30, 1932, Serial  
No. 627,117, and in Germany August 8, 1931

1 Claim. (Cl. 75—1)

This invention relates to surgical sewing needles, dental instruments and instruments of a like character or which have in use to comply with like requirements. Surgical sewing needles require above all considerable stiffness and extremely high elasticity in order that the surgeon, particularly when using curved surgical needles, can be completely certain of the path which the needle will take in the tissue to be sewn. Furthermore the elasticity must be so high that the eye when split for transversely inserting the thread can be opened without breaking, and after the insertion of the thread is automatically closed tightly and completely.

For these reasons surgical sewing needles have hitherto been successfully manufactured only from hardened steel, and all attempts to make such needles from stainless steels or corrosion-resistant alloys have so far failed, because no corrosion-resistant metallic material has, up to date, presented sufficient stiffness combined with sufficient elasticity.

The usual steel needles also have the disadvantage that if they are bent too much they break.

According to the invention surgical sewing needles are made from heat-treated nickel-beryllium alloys which may also include additions of other elements tending to increase the stiffness and elasticity. Extensive researches have shown that even binary nickel-beryllium alloys containing from 1 to 3% beryllium are equivalent in the heat-treated condition, as far as stiffness is concerned, to hardened and tempered carbon steel, and they even surpass this to a small extent. The elasticity also closely approaches that of hardened and tempered steel, while with proper fabrication nickel-beryllium alloys become substantially tougher than hardened and tempered steel.

In many cases the stiffness and elasticity of binary nickel-beryllium alloys are not good enough, for example for very thin and long needles. In such cases the stiffness and elasticity can be further increased by suitable additions of one or more of the elements chromium in amounts of up to 25%, molybdenum in amounts of up to 12%, tungsten in amounts of up to 18%, and cobalt up to 10%. The beryllium content of such ternary and complex alloys may actually be lower than in binary nickel-beryllium alloys for obtaining the same hardness and the same capacity of being improved by heat treatment; amounts of 0.3 to 2.5% are sufficient. Furthermore some of the nickel content, that is to say up to 25%, can be replaced by iron, but in no

case should the nickel content fall below 40% of the alloy if any corrosion attacks are to be met with certainty.

The alloys may advantageously contain from 0 to 25% of iron, 0.3 to 3% of beryllium, 10 to 20% of chromium, and either 4 to 10% of molybdenum or 2 to 5% of molybdenum and 3 to 8% of tungsten, or 2 to 5% of molybdenum, 3 to 8% of tungsten and 1 to 5% of cobalt, the remainder in each case being nickel except that small additions of such elements as manganese (about 0.5 to 3%), silicon (about 0.05 to 0.2%) and like elements may be included for the purpose of facilitating and improving the steps of fabrication by rolling and drawing. As one particularly suitable alloy for the manufacture of surgical sewing needles there may be mentioned an alloy containing from 0.3 to 3% beryllium, 15% chromium, 7% molybdenum, 15% iron and the remainder nickel.

A semi-circular surgical needle curved to a radius of 15 mm. made from the alloy mentioned above and having a stem thickness of from 1 to 1.2 mm. has a chord of 30 mm. measured from the point to the eye; such a needle can be bent until the distance between the point and the eye is 20 mm. and when released will spring back to the original chord of 30 mm. If, however, it is bent until the distance between the point and the eye is less than 15 mm., it takes a small permanent set, whereas a needle of hardened steel subjected to such a treatment would break. Needles with so-called spring eyes, that is eyes split longitudinally for the purpose of transverse introduction of the thread, behave entirely satisfactorily thanks to the remarkable elasticity and toughness of these alloys, and in fact the spring eyes of such needles break less easily than those of needles made of hardened steel. Surgical sewing needles hitherto made of corrosion-resistant materials have practically without exception been made without spring eyes, since the corrosion-resistant materials hitherto known and suitable for the manufacture of needles it was not possible to obtain sufficient resilience for spring eyes.

In the manufacture of surgical sewing needles from the said alloys it is advantageous to heat and quench for the last time before fabricating the needles to their final dimensions. Thereafter the needles are brought to their final dimensions by cold working which brings about a substantial increase in the hardness and elasticity, and only after the needles have been considerably hardened by cold working are they subjected to a tempering heat treatment. In this way it is pos-

sible to add together to a substantial extent the cold working hardness and the age hardening but in particular the toughness of needles thus made is substantially higher than that of needles which are heated, quenched and tempered only after the shaping has been completed.

The same considerations which have been discussed above in connection with surgical sewing needles apply also to other surgical needles, fine dental probes and other surgical and dental instruments and appliances. Specially fine dental probes, nerve needles and the like must have great toughness besides extremely high elasticity, because needles broken in the tooth practically always lead to loss of the tooth. Such probes and nerve needles are frequently also used

to introduce acids into the nerve canal of a tooth; the particularly high corrosion-resistance necessary for such instruments is present in needles made of nickel-beryllium alloys with addition of chromium and molybdenum which are substantially better in this respect than the binary nickel-beryllium alloys.

I claim:—

Surgical sewing needles, dental instruments and the like which require considerable stiffness and elastic hardness, made from an alloy containing iron up to 25%, beryllium 0.3 to 3%, chromium 10 to 20%, molybdenum 2 to 5%, tungsten 3 to 8%, and cobalt 1 to 5%, the remainder being nickel.

WILHELM ROHN.

20 90 25

25 95 100

30 100 105

35 110 115

40 115 120

45 120 125

50 125 130

55 130 135

60 135 140

65 140 145

70 145 150